

## UNITED STATES PATENT OFFICE

FRANCIS LOCKE, OF NORTH ATTLEBORO, MASSACHUSETTS, ASSIGNOR TO J. D. CROSBY COMPANY, OF PAWTUCKET, RHODE ISLAND, A CORPORATION OF NEW YORK

## METHOD OF MAKING POLISHED ANNEALED STAINLESS STEELS

No Drawing.

Application filed June 18, 1929. Serial No. 371,960.

The object of my invention is to provide a stainless steel and iron and the process of making the same. Whenever stainless steel or iron (for the purposes of this case called stainless steel) has been heated either to anneal, harden, or otherwise heat treat, it has been found that a discoloration or oxide is deposited on the surface which is removed with difficulty, and if the steel has a good finish before the heating treatment, this finish is destroyed by the attempts to remove the scale. My invention eliminates this difficulty and by my process, described below, stainless steels are heated in such a manner that they are discolored evenly and lightly and subsequently are restored to a bright, clean, oxide free, condition, free from pits, or other surface defects, such as would occur if the ordinary scale removing processes were employed, and with a finish approximately that which they had before the treatment. This finish is bettered further by light buffing.

This and other objects are accomplished by my invention, one embodiment of which is hereinafter more particularly set forth.

In the preferred embodiment of my invention, stainless steel of a suitable kind and character is passed cold through a series of rollers, the finishing rollers having highly polished surfaces so that after the last pass the sheet of metal emerges in a highly polished condition. This steel is then in such a hard condition, due to the action of the rollers, that it cannot be passed through dies or given similar treatment. If it be annealed in the ordinary way, the surfaces will be oxidized to such an extent that the high polish due to the rolling cannot be restored. My invention overcomes all difficulties and results in a product as above set forth.

My improved process and product will now be described in detail.

45

*The raw material*

The raw material may be hot rolled rods which must be clean, free from scale, black deposit stains, etc., and for convenience, these 50 rods may be annealed before rolling, although

this annealing is not essential. It is, however, desirable.

*Rolling*

The steel is cold rolled by giving many 55 light passes, each pass reducing the thickness by approximately .005". Wipers are used on the steel as it enters the rollers and also emery cloth so as to remove any dust or scale that may at any time appear on the 60 surface of this steel. The last rollings are between highly polished rollers. This imparts to the surface of the steel a high 65 polish and the cleaner the steel is kept, the better the polish and the better will be the ultimate product which is described below.

*Annealing*

The steel, in long strips, is drawn through an annealing furnace and kept at the proper 70 temperature while in the furnace, say substantially 1400° F., the exact temperature depending on the exact nature of the steel. From the furnace, this steel passes into a long cooling chamber, and out into the open air. 75 While being passed through the furnace and cooling chamber, the strip must not have any contact with any substance except a relatively movable substance, but must pass, with a continuous movement, over continuously 80 moving rollers, running with a peripheral velocity equal to the velocity of the strip, as nearly as may be. When the end of one strip is reached, another is secured to it, preferably by spot welding, and this follows 85 the first strip through the furnace and cooling chamber and this is continued while the apparatus is functioning. The velocity of the strip, when passing through the furnace and cooling chamber, is substantially 10 feet 90 per minute. The furnace atmosphere is maintained in the cooling chamber until near the exit end and so the strip is kept out of contact with air until near the end of the cooling chamber. The furnace atmosphere is 95 such that there is a slight oxidizing effect on the strip. This is important because it is exceedingly desirable that no deep or difficult scale be allowed to accumulate on the strip. Whatever does accumulate can be 100

readily removed and is readily removed by the next step of the process.

#### *Cleaning*

The scale or oxide on the steel from the annealing is removed as follows:

The steel is run continuously through a bath of substantially 10% sulphuric acid and while passing through this bath an electric current is passed through the strip, the current being a direct current of about 6 volts and the strip is the positive pole and the strip passes adjacent to metal plates which constitute the negative pole. These negative plates both lie over and below the strip. The combination of acid and electricity loosen the scale so that it is easily removed and brushed off before and after a bath through which the strip is passed. Thereafter the strip is drawn through a tank with water, which rinses the strip and withdraws all acids from the same and thereafter the strip is dried by being passed through sawdust or other suitable drying material. From this final drying the strip passes to a reel where it is allowed to accumulate.

Inferior results may be obtained if an alternating current be employed.

It is not essential that sulphuric acid be used, because any equivalent acid solution may be used, or a solution of salts, such as a sulphate of copper solution. Sulphuric acid of the kind, character and strength above indicated has been found suitable for the purpose of this process.

#### *The strip*

The strip, when processed as above described, has a finish, which when buffed is changed to a high polish, like that of a mirror. This polish may be obtained by buffing after the strip has been further processed by dies. This further processing would be impossible if the strip were not in an annealed condition prior to being passed through the dies.

With steels having an inferior initial finish, correspondingly inferior results are obtained although such finishes are superior to the prior art rolled finishes.

While I have shown and described one embodiment of my invention and the process of making the same, it is obvious that it is not restricted thereto but that it is broad enough to cover all products and processes that come within the scope of the annexed claims.

Having thus described my invention, what I claim is:

1. The process of making a polished, annealed, stainless steel which consists in rolling the stainless steel until it has the desired dimensions and polish and then passing the same through an annealing furnace and depositing a light oxide or scale on the same and thereafter removing this oxide or scale

by passing this steel through an acid bath, energized by electricity, the steel being the positive pole and thereafter washing or cleaning the loose scale resulting from the acid bath treatment.

2. The process of making a bright, clean, heat treated, stainless steel with its scale removed which consists in heating the steel in an atmosphere which will oxidize it slightly and evenly and then removing this oxide or scale by passing this steel through an acid bath, energized by electricity, the steel being the positive pole, and thereafter washing or cleaning the loose scale resulting from the acid bath treatment.

In testimony whereof, I have hereunto set my hand this 14th day of June, 1929.

FRANCIS LOCKE.

70

75

80

85

90

95

100

105

110

115

120

125

130